

## UNITED STATES PATENT OFFICE

GEORGE RIVAT, OF PATERSON, NEW JERSEY, ASSIGNOR TO CELANESE CORPORATION OF AMERICA, A CORPORATION OF DELAWARE

## DIFFERENTIALLY COLORED FABRIC AND METHOD OF MAKING THE SAME

No Drawing.

Application filed September 20, 1929. Serial No. 394,138.

This invention relates to the production of differentially colored fabrics by treating fabrics with an aniline black base after the application of a resist printing paste.

5 An object of my invention is to produce prints having dark or black backgrounds and lighter colored designs on fabrics containing organic derivatives of cellulose and particularly cellulose acetate. Another object 10 of my invention is to employ a resist printing paste containing vat dyestuffs in conjunction with a material containing aniline black base.

The production of prints having dark 15 backgrounds and lighter colored designs on fabrics containing organic derivatives of cellulose such as cellulose acetate, has presented serious problems. This is due to the fact that the dyestuffs that impart a dark color 20 to this fabric cannot be readily discharged by the ordinary discharge pastes used in the printing art. I have found, however, that if a paste containing an alkali and a metallic oxalate, with or without a vat dyestuff, is 25 locally applied to such fabric and then a material containing an aniline black base is applied thereto, after subsequent steaming or other oxidizing process, lighter colored 30 designs on black or dark backgrounds may be produced.

In accordance with my invention I produce lighter colored designs on dark or black backgrounds by the resist printing of fabric containing organic derivatives of cellulose 35 with a paste containing an oxalate and an alkali and preferably a swelling agent for the organic derivative of cellulose, which paste may or may not contain a vat dyestuff. After local application of the resist printing 40 paste, the fabric is padded with a material containing aniline black base and is then steamed to develop the color of the aniline black and also of the vat dyestuff if it is employed.

45 The fabric to be treated in accordance with my invention may contain yarns made of any organic derivative of cellulose such as organic esters of cellulose or cellulose ethers. Examples of organic esters of cellulose are 50 cellulose acetate, cellulose formate, cellulose

propionate and cellulose butyrate, while examples of cellulose ethers are ethyl cellulose, methyl cellulose and benzyl cellulose. The fabric need not necessarily consist wholly of 55 yarns made of these organic derivatives of cellulose, but may also contain yarns of other fibres such as cotton, silk or reconstituted cellulose.

The paste to be used for the resist printing, as stated before, contains a suitable alkali 60 such as potassium hydroxide, sodium hydroxide or alkaline salts such as sodium carbonate, etc. This paste also contains a metallic oxalate, such as sodium oxalate or potassium oxalate. In order to obtain suitable 65 penetration of the resist printing, I prefer to employ therein a swelling agent for the organic derivative of cellulose. Any suitable swelling agent may be employed, such as glycerin and/or ethyl alcohol, but if the 70 fabric is to be steamed before the application of the aniline black base, I prefer to use as swelling agent glycol derivatives that are less hydroscopic and better solvents for vat dyes, such as thiodiglycol sold under the 75 trade name of Glyezine A (general dyestuff) in order to avoid the running of the paste during the steaming.

Where white designs against dark background are desired, the resist paste will not 80 contain any dyestuff. However, if colored designs are desired, the resist paste will contain a suitable vat dyestuff. Examples of such vat dyestuffs are the algol colors, such as Algol red GGN (Color Index 1129) or the 85 indigosol colors such as Color Index Nos. 1178, 1184 and 1217. These vat dyestuffs are employed in the paste in suitably reduced condition.

The resist paste may be locally applied to 90 the fabric in any suitable manner, such as by printing with engraved or embossed rolls, or by brushing or spraying through stencils.

If the resist paste contains no color, or if 95 it contains a dyestuff of the indigosol type, it is not necessary to steam the fabric before padding with the aniline black. However, if the algol dyestuff range is used in the resist printing, the fabric is preferably steamed 100 for 5 minutes after the application of the re-

sist paste, if it is desired to obtain very deep shades.

After application of the resist printing paste, the fabric is padded with a paste containing aniline black base. This paste contains aniline in the form of its salt such as aniline hydrochloride or aniline sulphate rather than in the form of aniline oil. The paste contains an acid such as acetic acid, an oxidizing agent such as the chlorate of sodium or potassium, and a catalytic decomposition agent of the oxidizing salt, such as copper chloride.

After the padding of the aniline black base on the fabric, the fabric is subjected to steam under pressure for say about 5 minutes in a suitable ager such as the Mather Platt ager. This steaming causes oxidation of the aniline black base in those places where the resist has not been applied. However, the alkali and the metallic oxalate in the resist paste prevent the oxidation of the aniline black base where the resist paste has been applied. There is thus produced a discharge or printing effect of white or lighter colored design on a black or dark background. This steaming also develops the vat color, where it is employed, present in the resist paste.

In order further to illustrate my invention, specific details will be given in the following example.

A fabric consisting wholly of cellulose acetate yarn is printed with any of the following pastes.

#### Example A

For white resist effects the following paste may be employed.

|                | Parts |
|----------------|-------|
| Sodium oxalate | 7.5   |
| Water          | 19    |
| Glycerine      | 2     |
| Alcohol        | 4     |
| Gum tragacanth | 53.5  |
| Caustic soda   | 7.5   |
| Water          | 7.5   |

#### Example B

For a color resist employing an algol dye, the following may be used.

|                                         | Parts    |
|-----------------------------------------|----------|
| Sodium oxalate                          | 5.5      |
| Water                                   | 12.5     |
| Tragacanth paste                        | 31       |
| Caustic soda solution 50% concentration | 15 to 16 |
| Glyezine A                              | 4.1      |
| Algol paste reduced                     | 31       |

The algol paste reduced is made up as follows:

|                                       | Parts |
|---------------------------------------|-------|
| Algol red GGN paste 16% concentration | 300   |
| Sodium hydrosulphite                  | 250   |
| Potassium carbonate                   | 125   |
| British gum                           | 325   |

This mixture is heated at 50° C.

The color resist paste is allowed to stand 24 hours after preparation before it is used.

#### Example C

The following is an example of a color resist employing an indigosol color.

|                                         | Parts |
|-----------------------------------------|-------|
| Sodium oxalate                          | 6     |
| Water                                   | 13.2  |
| Tragacanth paste                        | 34    |
| Caustic soda solution 15% concentration | 17.3  |
| Glyezine A                              | 4.5   |
| Indigosol blue or Indigosol scarlet red | 9.3   |
| Water                                   | 15    |
| Caustic soda 50% solution               | 0.75  |

This paste is permitted to stand at least 24 hours after preparation before using.

If the fabric is printed with the white resist paste or the paste containing the indigosol colors, it is not necessary to steam before padding with the aniline black. If the algol dyestuff range is used in the printing paste, the fabric is steamed for 5 minutes before padding with the aniline black in order to obtain deep shades.

The fabric, after any of the above resist pastes have been applied thereto, is padded with an aniline black base paste, which is made by mixing equal parts of the two following solutions.

#### Solution A

|                       | Parts |
|-----------------------|-------|
| Aniline hydrochloride | 12.7  |
| Glacial acetic acid   | 2.5   |
| Water                 | 13    |
| Alcohol               | 10    |
| Tragacanth paste      | 32    |

#### Solution B

|                 | Parts |
|-----------------|-------|
| Sodium chlorate | 8     |
| Water           | 21    |
| Copper chloride | 0.8   |

After padding, the goods are steamed in an ager with steam under pressure for 5 minutes.

If the goods have been printed with a resist containing the algol colors, they are washed in lukewarm water and chromated for 5 minutes at 60 to 70° C. after which they are washed and soaped at 50 to 60° C.

If the goods have been printed with indigosol colors, the goods are washed at lukewarm temperatures with an aqueous solution containing 3 to 5 grams of sulfuric acid per litre for 10 minutes, after which they are given a chromate treatment for 1/2 hour at 50 to 60° C., then washed and scoured. The chromate treatment develops the colors of both the aniline black and of the vat dyestuffs.

It is to be understood that the foregoing detailed description is given merely by way of illustration and that many variations may

be made therein without departing from the spirit of my invention.

Having described my invention, what I claim and desire to secure by Letters Patent is:

1. Method of producing differential color effects comprising locally applying to a fabric containing an organic derivative of cellulose a material containing a swelling agent for the derivative of cellulose, an alkali and a metallic oxalate, applying a paste containing an aniline salt and an oxidizing agent and then steaming.
- 15 2. Method of producing differential color effects comprising locally applying to a fabric containing cellulose acetate a material containing a swelling agent for the cellulose acetate, an alkali and a metallic oxalate, applying a paste containing an aniline salt and an oxidizing agent and then steaming.
- 20 3. Method of producing differential color effects comprising locally applying to a fabric containing cellulose acetate a material comprising a swelling agent for the cellulose acetate, a vat dyestuff, an alkali and a metallic oxalate, applying a paste containing an aniline salt and an oxidizing agent, and then steaming.
- 25 4. Method of producing a differential color effect comprising printing a fabric containing cellulose acetate yarn with a resist paste containing sodium oxalate, sodium hydroxide, a swelling agent for cellulose acetate and a vat dyestuff in reduced state, drying,
- 30 then padding onto the fabric a paste containing an aniline salt, acetic acid, sodium chlorate and copper chloride, and then steaming.

In testimony whereof, I have hereunto subscribed my name.

GEORGE RIVAT.

45

50

55

60

65